

[72] Inventors **George E. Allen**  
**Boulder, Colorado;**  
**Glenn E. Allen, Rio Verde San Luis Potosi,**  
**Mexico**  
[21] Appl. No. **848,079**  
[22] Filed **Aug. 6, 1969**  
[45] Patented **Oct. 27, 1970**  
[73] Assignee **Allied Chemical Corporation**  
**New York, New York**  
**a corporation of New York**  
**Continuation-in-part of Ser. No.**  
**744,140, July 11, 1968, abandoned, which**  
**is a continuation of Ser. No. 478,858,**  
**Aug. 11, 1965, now Pat. No. 3,430,765**

[54] **BENEFICIATION OF FLUORSPAR ORES**  
**13 Claims, No Drawings**

[52] U.S. Cl. .... **209/11,**  
**209/167**  
[51] Int. Cl. .... **B63b 1/02,**  
**B03d 1/06**  
[50] Field of Search. .... **209/11,**  
**166, 167**

[56] **References Cited**  
**UNITED STATES PATENTS**  
1,914,695 6/1933 Lange..... **209/166**  
2,105,826 1/1938 Tartaron..... **209/166**  
3,138,550 6/1964 Woolery..... **209/166X**

3,382,976 5/1968 Mercade ..... **209/167**  
3,430,765 3/1969 Allen..... **209/166X**

*Primary Examiner—Frank W. Lutter*  
*Assistant Examiner—Robert Halper*  
*Attorneys—Gerard P. Rooney and Albert L. Gazzola*

**ABSTRACT:** "Acid-grade" fluorspar is recovered from fluorspar ores containing appreciable amounts of gangue minerals by a froth flotation treatment in a one-step fluorspar flotation circuit which comprises the steps of mixing crude fluorspar ore with water to form an aqueous pulp, adding to said aqueous pulp a water-soluble ferrous salt in an amount to provide between 0.2 and 0.8 pounds of ferrous salt per ton of crude fluorspar ore, adding to the pulp a collector for fluorspar, said collector selected from the group consisting of saturated fatty acids, mixtures of saturated and unsaturated fatty acids wherein the saturated fatty acid content of the mixture comprises at least about 30 percent of the total quantity of collector present and soaps of these acids or acid mixtures, and at least one depressant for gangue minerals selected from the group consisting of alkali metal silicates, alkali metal metasilicates, and quebracho, conditioning this mixture by heating said pulp to its boiling point with agitation while maintaining said pulp at a pH between about 8.0 and 9.0, subjecting said conditioned pulp to froth flotation thereby producing a froth rich in fluorspar and recovering in excess of 80 percent, based on the fluorspar from said froth. A further finding is that use of guar in this system increases the recovery of acid grade fluorspar.

## BENEFICIATION OF FLUORSPAR ORES

## CROSS-REFERENCE TO RELATED APPLICATIONS

This application is a continuation-in-part of U.S. application Ser. No. 744,140, filed July 11, 1968 now abandoned by George E. Allen and Glenn E. Allen for Beneficiation of Fluorspar Ores, which application in turn is a continuation-in-part of U.S. application Ser. No. 478,858, filed Aug. 11, 1965, now U.S. Pat. No. 3,430,765.

"Acid-grade" fluorspar, a term generally utilized to designate a concentrate containing at least 97 percent fluorspar ( $\text{CaF}_2$ ), is used in various chemical processes as a source of fluorine and hydrogen fluoride. The specifications as to allowable impurities vary with the industry but, in general, it is required that the fluorspar product be relatively free of gangue minerals such as quartz, calcite, clays and barite, as well as other accessory minerals including various sulfides such as galena, sphalerite, pyrite and chalcopyrite. Fluorspar ores as mined seldom meet the specifications either with respect to fluorspar content or freedom from impurities and suitable methods of concentration and ore separation must be employed to recover commercial "acid-grade" products from fluorspar ore. Although the beneficiation of fluorspar ores is readily effected by use of so-called "anionic" flotation reagents such as fatty acids, tall oils and the like, as well as various soaps thereof, the elimination of certain mineral impurities from the concentrate, thereby improving fluorspar grade, has been a difficult and costly task.

In the past a great many techniques have been employed to recover acid-grade fluorspar and generally these involve the addition of a plurality of special additives, e.g. sulfhydryl or xanthate collectors, which together with metallic salts subsequently interfere with the subsequent flotation of fluorspar. Additionally, it has been a common practice to have more than one flotation circuit to effectively remove the impurities from the fluorspar, thereby necessitating additional equipment which contributes to the milling costs in recovering an acid-grade fluorspar.

It has now been found that fluorspar ores containing in addition to fluorspar values appreciable quantities of gangue minerals may be concentrated to produce a fluorspar enriched concentrate having a fluorspar concentration of at least 97 percent in a one-step fluorspar flotation circuit by providing in the aqueous pulp of crude fluorspar ore minor amounts of a water-soluble ferrous salt, provided said ore does not contain the ferrous salt in the desired amounts. In issued Pat., U.S. Pat. No. 3,430,765, there was no recognition that if the fluorspar ore did not contain a water-soluble ferrous salt in an amount between 0.2 and 0.8 pounds per ton of crude fluorspar ore that the process disclosed in the patent provided only one advantage using the particular collector acids used, a lower silica content. However, it was found that when a water-soluble ferrous salt was added to the aqueous pulp both silica and carbonate could be held to acceptable limits while obtaining increased recovery of acid-grade fluorspar. This provides a definite depressing of sulfides, carbonates, silica and clay not obtainable if the water-soluble ferrous salt were not originally present or not added to the fluorspar ore prior to the conditioning step.

A further finding is that when guar is added to the aqueous pulp and conditioned in the presence of the particular collector acids employed in this process the clay slimes, barium sulfate and other gangue minerals are effectively blocked out, thus resulting in increased recovery of acid-grade fluorspar. The guar may be added with the normal depressants employed, e.g. alkali and alkaline silicates and metasilicates and quebracho.

When an aqueous fluorspar pulp is conditioned in the presence of the water-soluble ferrous salt, preferably in combination with guar, under the conditions of the present process, a froth rich in acid-grade fluorspar is selectively formed in a one-step fluorspar flotation circuit while gangue pyrite, are effectively separated from the fluorspar.

In accordance with the present invention, a fluorspar enriched concentrate having a fluorspar content of at least 97 percent is obtained from crude fluorspar ores containing in addition to fluorspar appreciable amounts of gangue minerals by mixing the crude ore with water to form an aqueous pulp, adding to the pulp a water-soluble ferrous salt in an amount to provide in the aqueous pulp about 0.2 to 0.8 pounds of ferrous salt per ton of crude ore, concentrating the pulp, adding to said pulp a collector for fluorspar selected from the group consisting of saturated fatty acids, mixtures of saturated and unsaturated fatty acids wherein the saturated fatty acid content of the mixture comprises at least about 30 percent of the total quantity of collector present and soaps thereof and adding at least one depressant for gangue minerals selected from the group consisting of alkali metal silicates, alkali metal metasilicates and quebracho, heating the pulp with agitation at its boiling temperature while maintaining said pulp at a pH between about 8.0 and 9.0, subjecting said pulp to froth flotation thereby forming a froth rich in fluorspar and recovering said fluorspar concentrate from the froth. Preferably, the guar is added to the pulp at this point.

In this process the fluorspar collector must be comprised, at least in part, of a saturated fatty acid or soap thereof is the one-step fluorspar flotation circuit for the selective flotation of "acid-grade" fluorspar is to be successful. Contrary to prior art procedures in which fatty acid collectors having a relatively high unsaturated fatty acid content, such as oleic acid and tall oil acids are conventionally employed, we have found that conditioning of the aqueous pulp in the presence of fully saturated fatty acid collectors or soaps thereof, present in an amount of at least 1.5 pounds per ton of ore milled, is essential in obtaining a fluorspar product of desired "acid-grade" purity. If desired, a portion of the saturated fatty acid collector may be replaced with an unsaturated fatty acid or soap thereof, provided that the saturated fatty acid content of the collector comprises at least about 30 percent, preferably between about 30 and 60 percent, of the total quantity of collector present. Moreover, by employing a saturated fatty acid collector, high recoveries, generally in excess of 80 percent of the fluorspar content present in the crude ore are effected. If the aqueous pulp is conditioned in the presence of unsaturated fatty acid collectors alone, such as oleic acid, or in the presence of a commercial preparation containing predominantly unsaturated fatty acids, substantially lower recoveries of the fluorspar content of the crude ore are obtained and the fluorspar concentrate resulting from such a one-step flotation procedure is contaminated with excessive amounts of minerals, precluding obtainment of an "acid-grade" product.

The fatty acids and soaps thereof employable as collectors in the present process are well-known materials. Included within the term soaps are the alkali metal and alkaline earth metal soaps such as sodium, potassium, calcium, magnesium and aluminum soaps. Suitable saturated fatty acids include acids containing from about 4 to 22 carbon atoms, preferably 12 to 18 carbon atoms, in the molecule such as palmitic acid, lauric acid, stearic acid, commercially available preparations containing minor amounts of unsaturated fatty acids such as Hyfac 423, Hyfac 425, Hyfac 400 made by Emery Industries, Inc.; and Swift 55, Swift 62, Swift RG made by Swift and Company, etc., all of which contain at least about 80 percent saturated fatty acids. Accordingly, as used in the present case, the term "saturated fatty acid" is intended to include such mixtures of fatty acids as are found in commercial products. If desired, unsaturated fatty acids containing from about 12 to 20 carbon atoms in the molecule such as crude and purified oleic acid, palmitoleic acid, linoleic acid, distilled tall oils, commercial preparations containing a major amount of unsaturated fatty acids such as Acintol FA1 tall oil fatty acid and 70 Acintol FA2 tall oil fatty acid produced by the Arizona Chemical Company; Emersol 211 low-titer oleic acid, Emersol 531 distilled tallow fatty acid and Emтал 665 fractionated tall fatty acid made by Emery Industries, Inc., etc., may be used in conjunction with the saturated fatty acids. Although 75 the amount of fatty acid collector used may be varied widely,

amounts of about 1.5 to 5 pounds per ton of ore milled are generally satisfactory. It is necessary, however, when commercial saturated fatty acid preparations and mixtures of saturated and unsaturated fatty acids are employed that the saturated fatty acid content of the collector comprise at least about 30 percent, preferably between about 30 and 60 percent, of the total quantity of collector present to effect selective flotation of the fluorspar values contained in the ore. The preferred collector is comprised of mixtures of saturated and unsaturated fatty acids having from 12 to 18 carbon atoms and having a saturated fatty acid content between about 30 and 60 percent.

In effecting the one-step fluorspar flotation circuit for the recovery of the acid-grade fluorspar values contained in the crude ore in accordance with the present process, it has been found necessary to add at least one of an alkali metal silicate, alkali metal metasilicate, such as sodium silicate or sodium metasilicate, or quebracho in conjunction with the fatty acid collector during the conditioning step of the process. In addition to these reagents guar has been found unexpectedly effective in combination with the use of the ferrous salt added. While certain of these reagents may act together with the pH regulator as an alkalinity modifier, under the conditions of the present process such reagents also serve as depressants for gangue minerals and disperse slimes, thereby permitting selective flotation of the fluorspar values by the fatty acid collector. The quantity of additive employed may also be varied widely and, in general, satisfactory results are obtained when the depressant is used in an amount of from about 0.1 to about 6, preferably from about 0.2 to about 5 pounds per ton of ore milled. The amount of silicate generally employed may range from about 2 to 6 pounds per ton of ore milled. The amount of quebracho used is generally between about 0.2 and 0.8 pounds per ton of crude ore, but can vary widely.

As mentioned above, it has been found that guar when added in combination with the water-soluble ferrous salt effectively blocks out clay slimes, barium sulfate and other gangue minerals and result in increased fluorspar recovery. The guar suppresses the slimes and gangue so that it does not float when the collector acid(s) is added. The guar can be added to the grinding mill or conditioner at or near the same point of addition as the water-soluble ferrous salt and the depressants employed. Preferably, the guar is added to the aqueous pulp prior to the conditioning step so that the guar and aqueous pulp are for about 2 to 10 minutes prior to the addition of the collector acid(s). However, in some applications the addition of the guar simultaneously with the conditioning agents has been found effective. Guar is compatible with the other agents used in the flotation process of this invention and may be added as a dry powder or as an aqueous dispersion in amounts of about 0.1 to 0.7, preferably 0.2 to 0.5, pounds per ton of ore milled with smaller amounts adequate for the higher grade fluorspar ores and increased amounts for the lower grade ore.

During the conditioning of the aqueous pulp it has been found that in order to obtain a fluorspar concentrate of the desired purity the conditioning should be effected at its boiling temperature at a pH in the range of about 7.0 to 10.0, preferably 8.4 to 8.8, for a minimum period of time, generally at least about 5 minutes. After boiling the pH will be lowered and will vary from about 7 to 9.0, with a pH of 8.4 to 8.8 considered optimum. Unless conditioning is effected at the pH ranges, temperature and time specified, substantial quantities of the minerals present in the pulp will be floated together with the desired fluorspar. Since different fluorspar ores will give varying pH values when slurried in water, it is usually necessary to adjust the pH of the pulp with a conventional pH regulating reagents. The pH regulator may be added to the pulp at any time before completion of the conditioning stage of the process but it is preferred to add the requisite quantities of pH regulator necessary to maintain the pH within the stated values simultaneously with the fatty acid collector and gangue mineral depressant prior to conditioning of the pulp. A pulp of too low pH may be brought to the desirable pH by addition of

an alkaline reagent such as an alkali metal hydroxide or carbonate, e.g. sodium hydroxide or sodium carbonate. In some instances, the addition of sufficient quantities of fatty acid collector and gangue mineral depressant will give a pulp of suitable pH without the addition of any other pH modifying agent.

The composition of the ores treatable in accordance with the present invention generally comprises from about 40 to 90 percent calcium fluoride, up to about 50 or more percent gangue minerals such as quartz and calcite, up to about 15 percent sulfide minerals including galena, sphalerite and pyrite, minor amounts normally less than about 3 percent of complex metallic salt contaminants and minor quantities of other impurities.

In practicing the invention, the ore is first prepared for flotation by conventional methods. In accordance with these methods, the dry ore is crushed and ground sufficiently to pass a 48 mesh screen. The fineness of the grind may vary from 60 to 90 percent 200 mesh depending on the locking characteristics of the ore. However, substantially complete liberation of the fluorspar from the gangue is required for a satisfactory separation and the fineness of grind should be selected accordingly. The ground ore is then mixed with sufficient quantities of water in a ball mill to form an aqueous pulp having a solids content of about 60 to 80 percent by weight based on the weight of the pulp. Although local water supplies may ordinarily be employed in forming the pulp, softened water having a total hardness of not greater than about 200 p.p.m. is preferred since the use of softened water reduces the fatty acid requirements in collection of the fluorspar rich froth. If the crude ore does not contain a water-soluble ferrous salt such as ferrous sulfate it is added in amounts to provide about 0.2 to 0.8 pounds per ton of crude ore.

Thereafter, the solid particles contained in the aqueous pulp or slurry are classified to produce a pulp having a particle size suitable for flotation, generally ranging from about 48 mesh to 10 microns. The aqueous pulp is then fed to a concentrator or thickener to form a pulp having a solids content of about 35 to 45 percent by weight based on the weight of the pulp, and the water obtained as a result of thickening of the pulp is withdrawn as waste from the concentrator by any conventional manner as by decantation. Preferably, it is at this point in the process at which the guar is added. If desired, any commercial flocculating or agglomerating agent may be employed in the concentrator to assist in settling of the pulp. In accordance with the present process, the complex metallic salt contaminants present in the pulped ore are solubilized in the waste water and a large portion of the contaminants are removed therewith when the pulp is thickened in the concentrator. This contrasts with conventional procedures employing a preliminary sulfide flotation circuit wherein, under the conditions employed, the complex metallic salt contaminants are precipitated, carried over into the fluorspar froth flotation circuit and therein interfere with the selective flotation of the desired fluorspar values. In the process of this invention the amount of contaminants carried over is sufficiently small so as not to interfere with the selective flotation.

After the aqueous pulp has been classified and concentrated to produce a pulp having a particle size and solids content suitable for flotation, the pulp is fed into a conditioning tank where it is heated to its boiling point with agitation. The boiling temperature of the pulp may be higher or lower than 212°F. depending upon the atmospheric pressure at the point of location of the operation. Although the practice of the present invention is not limited to any particular order of addition of the separate conditioning reagents, it is preferred, however, to properly condition the pulp after the requisite quantities of fatty acid collector and gangue depressant have been added to the pulp together with suitable quantities of pH regulator to adjust the pH of pulp to a value between 7.0 and 10.0, preferably between 8 and 9. If desired, a portion of the requisite quantity of the fatty acid collector and gangue depressant may be added to the pulp prior to heating and the remaining quantities may then be added to the pulp either in-

termittently or continuously during conditioning at the boiling temperature of the pulp.

Although any conventional apparatus having external or internal heating means may be employed to condition the pulp, a preferred procedure involves introducing sufficient quantities of steam into the conditioning tank as through pipes discharging below the pulp level to bring the pulp to its boiling temperature. Sufficient conditioning of the pulp is normally achieved as the pulp is brought to its boiling temperature with agitation. However, it is generally necessary to condition the pulp at its boiling temperature for a period of 5 to 60 minutes, preferably 15 to 45 minutes, especially if high recoveries of the fluorspar content contained in the pulped ore are to be realized. After conditioning of the pulp has been completed, the pulp, at or near its boiling temperature, or after being allowed to cool to ambient temperatures, is then froth floated by customary mechanical or pneumatic methods to produce an enriched fluorspar froth and a tailings product essentially free of fluorspar and containing the gangue materials and sulfide minerals. In general, the solids content of the pulp after conditioning is reduced to about 20 to 30 percent by weight based on the weight of the pulp.

The froth product may contain some quartz, calcite, or other gangue materials collected with the fluorspar in the initial frothing operation. The froth is generally refloated to recover the fluorspar and reject the remaining gangue materials. One or more such cleaning operations generally suffices to yield final fluorspar enriched concentrates having a fluorspar content of at least 97 percent and essentially free from gangue and other impurities. Additional reagents, such as a small quantity of alkali metal silicate or quebracho may be used in the cleaning operations to facilitate rejection of the gangue impurities. The tailings material, resulting from the cleaning operations, may be recycled to preceding flotation steps or other convenient points in the flotation or grinding circuit for retreatment, or may be rejected as waste.

As mentioned above, the water-soluble ferrous salt should be present in, or added to the aqueous pulp preferably before concentrating the pulp, in an amount to provide about 0.2 to about 0.8 pounds of ferrous salt per ton of crude ore milled. One way which has successfully been used achieving this in the pulp is to add to the pulp a sufficient amount of a 10 percent by weight aqueous solution of the ferrous salt, such as ferrous sulfate, to provide an amount of ferrous salt within the above limits. The upper limit of the specified range is dictated by economics and thus natural ores having higher water-soluble ferrous salt contents can be used without difficulty.

The water-soluble ferrous salts are believed to function by the association of the ferrous ion with the gangue materials, giving the gangue materials a greater affinity for water. The combination of the use of a water-soluble ferrous salt with a collector comprising at least 30 percent saturated fatty acids as specified above has been found to yield unexpectedly superior acid grade fluorspar recovery. Although the water-soluble ferrous salt is preferably added to the pulp at the ball mill, it can also be added with the collector if desired.

It will be apparent to anyone skilled in the art that the process of this invention can be operated as a batch, intermittent batch or as a continuous process by means of recognizable variations in the apparatus and use thereof.

The following examples, while not intended to limit the scope of the invention, are illustrative of the benefits derived from the practice thereof. The ores of Examples 1 and 2 were found to contain sufficient ferrous salt so as not to require the addition of the salt. These Examples exemplify the process of U.S. Pat. No. 3,430,765.

#### EXAMPLE 1

A crude broken fluorspar ore consisting essentially of fluorspar associated with appreciable quantities of a siliceous gangue composed predominantly of quartz, metallic sulfides including galena, sphalerite and pyrite, and minor amounts of

sulfur (present as complex metallic salt contaminants) was obtained from a Colorado deposit. The ore had been stored underground in the mine for a period of about 52 weeks after being mined. The crude ore assayed 46.9 percent  $\text{CaF}_2$ , 32.2 percent  $\text{SiO}_2$ , 6.0 percent metallic sulfides, 2.5 percent  $\text{CaCO}_3$ , and 2.0 percent S. overflow

The crude ore was subjected to staged crushing, screening, wet grinding and classifying operations to produce an aqueous pulp containing solids having a particle size such that 67 percent passed through a 200 mesh screen. The pulp discharging from the ball mill wherein the ore was wet ground had a solids content of 68 percent, based on the weight of the pulp, and the classifier overflow was maintained to produce a pulp having a solids content of 16 percent, based on the weight of the pulp. The water used for wet grinding of the ore contained the equivalent of 100 p.p.m. total hardness. Separan, a commercial flocculating agent, was added to the classifier overflow product in an amount equivalent to 0.04 pound per ton of ore milled to assist in settling the pulp.

The aqueous pulp was then thickened by decantation to produce a pulp having a solids content of about 40 percent, based on the weight of the pulp. The thickened pulp was then transferred to a conditioning tank to which there was added the equivalent of 1.9 pounds per ton of Hyfac 400, a commercial hydrogenated fatty acid comprised of about 90 percent saturated fatty acids containing from 14 to 18 carbon atoms, the equivalent of 2.3 pounds per ton of Acitol FA2, a tall oil fatty acid comprises of about 50 percent oleic acid and 46 percent linoleic acid, the equivalent of 4.7 pounds per ton of sodium silicate and sufficient sodium carbonate (equivalent of 14.0 pounds per ton) to bring the pulp to a pH of about 8.8. The pulp was then conditioned at its boiling temperature (201°F.) by introducing steam at a temperature of 352°F. and 75 p.s.i. through pipes discharging below the pulp level for a period of 20 minutes.

After conditioning, sufficient water was added to the pulp to produce a pulp having a solids content of about 25 percent by weight based on the weight of the pulp. The diluted pulp was then continuously fed into the first cell of a bank of flotation cells to which air was continuously introduced, thereby resulting in formation of a compact, heavily mineralized fluorspar froth. The underflow comprising the tailings was rich in gauge and sulfide materials. The rougher froth was then cleaned by refloating in a series of flotation cells. The final fluorspar concentrate assayed 97.07 percent  $\text{CaF}_2$ , 0.94 percent  $\text{SiO}_2$ , 0.85 percent  $\text{CaCO}_3$ , 0.002 percent metallic sulfides and no complex metallic salt contaminants and accounted for a recovery of 90.8 percent of the fluorspar in the ore.

#### EXAMPLE 2

A crude fluorspar ore assaying 51.1 percent  $\text{CaF}_2$ , 31.0 percent  $\text{SiO}_2$ , 3.0 percent  $\text{CaCO}_3$ , 6.0 percent sulfide minerals and 2.0 percent S (present as complex metallic salt contaminants) was processed for recovery of fluorspar values contained therein in accordance with the procedure described in Example 1 except that essentially saturated fatty acids, Hyfac 400, present in an amount equivalent to 4.0 pounds per ton of ore milled, was used as the sole collector.

In this example, sodium silicate was added to the concentrated pulp together with the hydrogenated fatty acid collector in an amount equivalent to 3.2 pounds per ton of ore milled, and sufficient sodium carbonate (equivalent to 18.7 pounds per ton) was added to bring the pH of the pulp to a value of 8.4. The pulp was conditioned, floated and cleaned in the same manner as in the preceding example. The final fluorspar concentrate assayed 98.6 percent  $\text{CaF}_2$ , 0.50 percent  $\text{SiO}_2$ , 0.34 percent  $\text{CaCO}_3$ , 0.003 percent metallic sulfides and no complex metallic salt contaminants and represented a recovery of 83.3 percent of the fluorspar in the ore.

Example 3 exemplifies the process of the present invention.

## EXAMPLE 3

A crude fluorspar ore assaying 87.23 percent  $\text{CaF}_2$ , 4.68 percent  $\text{SiO}_2$  and 4.66 percent  $\text{CaCO}_3$  was processed for recovery of fluorspar values contained therein in accordance with the following procedure.

The ore was subjected to staged crushing and screening. The crushed product was then wet ground in a ball mill with the addition of ferrous sulfate in an amount equivalent to 0.275 pounds per ton to produce an aqueous pulp containing solids having a particle size such that 89 percent passed through a 200 mesh screen. The pulp discharging from the ball mill wherein the ore was wet ground had a solids content of 70 percent, based on the weight of the pulp, and the classifier overflow was maintained to produce a pulp having a solids content of 49 percent, based on the weight of the pulp. The water used for wet grinding of the ore contained the equivalent of 190 p.p.m. total hardness. Separan, a commercial flocculating agent was added to the concentrator in an amount equivalent to 0.04 pounds per ton of ore milled to assist in settling the pulp. The aqueous pulp was then thickened by decantation. The thickened pulp, having a solids content of about 58 percent based on the weight of the pulp, was then transferred to a combination boil-conditioner tank. At this point there were added amounts equivalent to 2.2 pounds per ton of stearic fatty acid, 3.3 pounds per ton of Acitol FA2 (see Example 1) and 0.97 pounds per ton sodium carbonate. The pulp was then conditioned at its boiling temperature (207°F.) by introducing steam through coils in the conditioner for a period of 20 minutes. After conditioning, sufficient water was added to the pulp to produce a pulp having a solids content of about 30 percent by weight based on the weight of the pulp. At the conditioner discharge, quebracho in an amount equivalent to 0.18 pounds per ton of crude ore and sodium silicate in an amount of 3.67 pounds per ton of crude ore were added to the diluted pulp which was fed into the first cell of a bank of flotation cells to which air was continuously introduced, thereby resulting in formation of a compact, heavily mineralized fluorspar froth. The underflow comprising the tailings was rich in gangue. The rougher froth was then cleaned by refloating in a series of flotation cells where quebracho was added in two stages in amounts equivalent to 0.37 pounds per ton in each stage to further depress the carbonate gangue minerals. The final fluorspar concentrate assayed 97.48 percent  $\text{CaF}_2$ , 1.03 percent  $\text{SiO}_2$  and 1.03 percent  $\text{CaCO}_3$  and accounted for a recovery of 91.0 percent of the fluorspar in the ore.

Substantially similar results may be obtained with employment of sodium metasilicate as a conditioning agent and sodium hydroxide as a pH regulator.

## EXAMPLE 4

In order to demonstrate the benefit of adding ferrous sulfate to a fluorspar ore which did not originally contain the salt in the desired amounts two series of runs were conducted on these fluorspar ores. The ores which were processed in this example following the procedure described in Example 3 analyzed as follows:

|                 | Percent |
|-----------------|---------|
| $\text{CaF}_2$  | 89.05   |
| $\text{SiO}_2$  | 5.94    |
| $\text{CaCO}_3$ | 3.33    |

In one of the series of runs (3 tests) no ferrous sulfate was added. In the other series of runs (7 tests) approximately 0.25 to 0.33 pounds of ferrous sulfate per ton of fluorspar ore was added to the ore during the grind circuit. The process conditions of Example 3 were employed. The results of these tests were averaged and are presented below:

|                           | No Ferrous Sulfate <sup>1</sup> | Ferrous Sulfate Added <sup>2</sup> |
|---------------------------|---------------------------------|------------------------------------|
| $\text{CaF}_2$ , percent  | 97.35                           | 97.63                              |
| $\text{SiO}_2$ , percent  | 0.89                            | 1.01                               |
| $\text{CaCO}_3$ , percent | 1.43                            | 0.99                               |
| Recovery, percent         | 86.60                           | 90.46                              |

<sup>1</sup> Average of three (3) tests.

<sup>2</sup> Average of seven (7) tests.

From these data it may be observed that the use of ferrous sulfate resulted in an increase in grade of the fluorspar produced and a 3.8 percent increase in recovery.

## EXAMPLE 5

In order to demonstrate the effectiveness of guar as an auxiliary gangue depressant in the practice of the present process a series of tests were conducted following the procedure of Example 3, except in one series of runs guar was present in addition to the quebracho and sodium silicate depressants. About 0.30 pounds of guar per ton of ore was added to the aqueous pulp during the grind circuit of the other series of runs. Ferrous sulfate was present in both series of runs in an amount of about 0.25 pounds per ton of ore. The results of these runs are presented below:

(1) 1 Average of three (3) tests

(2) Average of seven (7) tests

## FLUORSPAR ORE ANALYSIS

|                           | A     | B     | C     |
|---------------------------|-------|-------|-------|
| $\text{CaF}_2$ , percent  | 76.00 | 87.55 | 89.05 |
| $\text{SiO}_2$ , percent  | 14.23 | 8.24  | 5.94  |
| $\text{CaCO}_3$ , percent | 6.62  | 2.52  | 3.33  |

## RUNS WITHOUT GUAR ADDITION

|                           | A     | B     | C     | Average |
|---------------------------|-------|-------|-------|---------|
| $\text{CaF}_2$ , percent  | 97.57 | 97.61 | 97.12 | 97.43   |
| $\text{SiO}_2$ , percent  | 0.81  | 1.34  | 1.26  | 1.14    |
| $\text{CaCO}_3$ , percent | 0.81  | 0.70  | 1.29  | 0.93    |
| Recovery, percent         | 82.20 | 90.50 | 95.00 | 89.23   |

## RUNS TO WHICH GUAR WAS ADDED

|                           | A     | B     | C     | Average |
|---------------------------|-------|-------|-------|---------|
| $\text{CaF}_2$ , percent  | 97.58 | 97.50 | 97.34 | 97.47   |
| $\text{SiO}_2$ , percent  | 1.33  | 1.39  | 1.27  | 1.33    |
| $\text{CaCO}_3$ , percent | 0.53  | 0.70  | 0.89  | 0.70    |
| Recovery, percent         | 95.90 | 97.17 | 97.50 | 96.85   |

From these data it may be observed that the presence of guar in addition to the quebracho and sodium silicate consistently gave an acid-grade fluorspar concentrate in high yields.

The results of the above-described flotation procedures may also be reproduced on other fluorspar ores containing appreciable quantities of gangue minerals. Metallic sulfides, quartz and silicate minerals including feldspar, clay and associated iron oxide are readily retarded by the process of the present invention thereby enabling a good recovery of the fluorspar as "acid-grade" concentrates.

We claim:

1. A process for producing a fluorspar enriched concentrate having a fluorspar content of at least 97 percent from a crude fluorspar ore containing in addition to fluorspar appreciable amounts of gangue minerals which consist essentially of a one-step fluorspar flotation circuit comprising mixing the crude ore with water to form an aqueous pulp, adding to the aqueous

pulp a water-soluble ferrous salt in an amount sufficient to provide between 0.2 and 0.8 pounds of ferrous salt per ton of crude fluorspar ore milled, at least one depressant for gangue minerals selected from the group consisting of alkali metal silicates, alkali metal metasilicates and quebracho, and a collector of fluorspar, said collector selected from the group consisting of saturated fatty acids, mixtures of saturated and unsaturated fatty acids wherein the saturated fatty acid content of the mixture comprises at least about 30 percent of the total quantity of collector present, and soaps thereof, conditioning this mixture by heating said pulp to its boiling point with agitation while maintaining said pulp at a pH between about 7.0 and 10.0, subjecting said pulp to froth flotation, thereby producing a froth rich in fluorspar and recovering in excess of 80 percent based on the fluorspar content in the crude ore, of acid-grade fluorspar from said froth.

2. The process of claim 1 wherein the fluorspar ore additionally contains at least one of metallic sulfides and metallic salt contaminanats.

3. The process of claim 1 wherein the water-soluble ferrous salt is ferrous sulfate.

4. The process of claim 1 wherein the saturated fatty acid content of the collector is present in an amount of at least 1.5 pounds per ton of ore milled.

5. The process of claim 4 wherein the collector is a mixture of saturated and unsaturated fatty acids containing from 12 to 18 carbon atoms and the depressant is an alkali metal silicate.

6. The process of claim 1 wherein the aqueous pulp additionally has added to it prior to conditioning by heating a minor amount of guar.

7. The process of claim 6 wherein guar is added to the aqueous pulp prior to the addition of the collector.

8. The process of claim 7 wherein the guar is in contact with the aqueous pulp for about 2 to 10 minutes prior to the addition of the collector.

9. The process of claim 1 wherein guar is added to the aqueous pulp in an amount between 0.1 and 0.7 pounds per ton of fluorspar ore.

15 10. The process of claim 1 wherein the collector is a saturated fatty acid containing from 12 to 18 carbon atoms.

11. The process of claim 1 wherein the collector is a mixture of saturated and unsaturated fatty acids containing from 12 to 18 carbon atoms.

20 12. The process of claim 1 wherein the depressant is an alkali metal silicate.

13. The process of claim 1 wherein the depressant is a mixture of an alkali metal silicate and quebracho.